

Aug. 17, 1943.

W. M. CAMP

2,326,832

PLASTIC TRAVELER

Filed March 31, 1942

PLASTICIZED CELLULOSE ESTER



Fig. 1.

PLASTICIZED CELLULOSE ESTER



PLASTICIZED CELLULOSE ESTER



Fig. 3.

PLASTICIZED CELLULOSE ESTER



Fig. 4.

INVENTOR.  
William M. Camp

BY

Jeffre, Eule, Burgos  
ATTORNEYS

## UNITED STATES PATENT OFFICE

2,326,832

## PLASTIC TRAVELER

William M. Camp, Glen Ridge, N. J., assignor to  
 The Clark Thread Company, Newark, N. J., a  
 corporation of New Jersey

Application March 31, 1942, Serial No. 437,042

11 Claims. (CL 57—125)

This invention relates to travelers which are used on spinning and twisting frames in the textile industry.

In the past, travelers have been made of either steel or bronze, the bronze being used mostly on wet twisting, where the presence of water makes it undesirable to use steel. These travelers rotate around the ring at a high speed, and in the case of twisting where the drag on the traveler is heavy it is necessary to provide lubrication between the traveler and the ring, this taking the form of an oil or grease. Even under conditions of good lubrication, wear takes place on the traveler and also on the ring and the fine particles of metal which are worn off become embedded in the grease and are subsequently oxidized and thus form visible stains on the yarns or threads. These stains consist of oxides, carbonates, soaps, etc., of the respective traveler and ring metals, and are very difficult to remove in the ordinary processes of kier-boiling and bleaching.

Many attempts have been made to make travelers of materials, other than steel and bronze, using materials including hard rubber and glass. These materials, however, have not been satisfactory because of their brittleness and poor resistance against wear.

It is an object of this invention to provide a traveler possessing properties which have long been sought, including the following:

1. A longer life than steel or bronze travelers.
2. Requiring less lubrication than steel or bronze travelers or no lubrication.
3. Producing little or no wear on the steel ring and therefore obviating the contamination of the yarn or thread referred to above.
4. Corrosion resistance, to avoid corrosion in wet twisting.

The invention will be further described by reference to the accompanying drawing, in which

Fig. 1 shows one type of conventional ring with a traveler mounted thereon;

Fig. 2 shows a traveler for use with the ring of Fig. 1;

Fig. 3 shows another type of conventional ring with a traveler mounted thereon; and

Fig. 4 shows a traveler for use with the ring shown in Fig. 3.

In accordance with the generic aspect of this invention, travelers are made from plasticized cellulose esters in general. In accordance with a more specific aspect of this invention, mixed esters in general are used. Certain species are preferred, to wit, cellulose nitrate, cellulose ace-

tate and cellulose acetate butyrate, i. e., the mixed cellulose ester of acetic and butyric acids. Since plasticized cellulose esters for the manufacture of molded or machined articles are <sup>5</sup> well known, it is not necessary to describe the composition and properties thereof. The proportion and kind of plasticizer, the proportion and kind of acid or acids combined with the cellulose and the kind of cellulose employed for esterification are details known to the art of making plastic cellulose esters and may be varied within the skill of this art, in the light of the present invention, to secure a cellulose ester product adapted to meet the preferred criteria of this invention. These, briefly, are resiliency, toughness, shock resistance, abrasion resistance and corrosion resistance. Resiliency is desired because the jaws of the traveler are usually sprung apart in mounting on the ring. Toughness and shock or impact resistance are desired so that breakage will not occur. Abrasion resistance is desired to avoid undue wear. Corrosion resistance is desired to avoid corrosion in wet twisting.

<sup>25</sup> Having obtained the plasticized cellulose ester stock desired, the traveler is made therefrom by molding or machining from extruded or pre-molded stock. No details as to the structural form of the traveler are necessary because the various shapes and forms of travelers are well known now, and no details as to the process of molding or machining need be specified since the art of molding and machining cellulose esters is well known.

<sup>30</sup> <sup>35</sup> However, in some cases, it may be desired to provide the traveler with a metallic core, i. e., make a traveler having a metallic core and a wearing surface comprising or composed essentially of a cellulose ester. This may be done, for example, by using a steel or alloy core or insert and molding the cellulose ester composition around said core so that the latter is embedded in the resulting molded product.

I claim:

- <sup>40</sup> 1. A traveler the wearing surface of which comprises a plasticized cellulose ester.
2. A traveler for wearing surface of which comprises a plasticized cellulose nitrate.
3. A traveler the wearing surface of which comprises a plasticized cellulose acetate.
4. A traveler the wearing surface of which comprises a plasticized cellulose acetate butyrate.
- <sup>45</sup> 5. A traveler the wearing surface of which comprises a plasticized mixed cellulose ester.

6. A traveler consisting essentially of a plasticized cellulose ester.
7. A traveler consisting essentially of a plasticized cellulose nitrate.
8. A traveler consisting essentially of a plasticized cellulose acetate.
9. A traveler consisting essentially of a plasticized cellulose acetate butyrate.
10. A traveler consisting essentially of a plasticized mixed cellulose ester.
11. A traveler having a metallic core and a wearing surface composed essentially of a plasticized cellulose ester.

WILLIAM M. CAMP.